

Sept. 28, 1965

R. S. OWENS ET AL

3,208,940

LUBRICATING COMPOSITIONS AND METHODS OF LUBRICATING

Filed March 19, 1962



Inventors:  
Robert S. Owens;  
Leon E. St. Pierre,

by Joseph T. Cohen

Their Attorney.

3,208,940

LUBRICATING COMPOSITIONS AND METHODS  
OF LUBRICATING

Robert S. Owens, Latham, and Leon E. St. Pierre, Schenectady, N.Y., assignors to General Electric Company, a corporation of New York

Filed Mar. 19, 1962, Ser. No. 180,883

12 Claims. (Cl. 252—45)

This application is a continuation-in-part of our earlier abandoned application Serial No. 101,918, filed April 10, 1961, and assigned to the same assignee as the present invention.

This invention is concerned with improved lubricants, and uses of these materials as lubricants for various contacting metallic surfaces. More particularly, the invention relates to lubricants and surfaces lubricated with such lubricants in which one of the surfaces is a metal composition particularly aluminum or a composition containing at least 50% by weight aluminum, for instance, alloys of aluminum, the said lubricants comprising a mixture of ingredients comprising (1) a long chain olefin of at least 10 carbon atoms and (2) an organic compound containing a polar group, a linear long chain, saturated aliphatic radical having at least 11 carbon atoms, and a straight chain lower alkyl group containing from 1 to 3 carbon atoms separated from the long chain radical by the polar group.

For purposes of brevity, the term "aluminum" or "aluminum composition" is intended to include not only aluminum itself, but also compositions in which the aluminum is present in an amount equal to at least 50% of the total weight of the composition, as, for instance, aluminum alloys, etc.

Attempts have been made in the past to effect lubrication of aluminum surfaces. Thus, it has been desired to effect lubrication of relatively moving surfaces in which one of the surfaces is a metal composition containing at least 50% by weight aluminum, for instance, pure aluminum, alloys of aluminum, etc. The lubrication of such aluminum surfaces is especially difficult in cases where extreme pressure conditions exist requiring lubrication under boundary lubricating conditions, i.e., actual solid-to-solid contact, for instance, as may be found in a bearing before a hydrodynamic film of lubricant is created or where new solid surfaces are being generated, for example, in the shaping of a metal wire by drawing through a die, in the cutting of aluminum metal, for example, in a lathe or punch-press, the shaping of aluminum metal, for example, by stamping, extrusion, spinning, cold-rolling, etc. For convenience, this type of lubrication is hereinafter referred to as "boundary lubrication." Under such conditions, it has been found that aluminum compositions are lubricated with great difficulty due to the fact that under extreme pressure conditions of boundary lubrication, the aluminum surface tends to score, gall, or seize, even when great care is exercised. To the best of our knowledge, no previous lubricant has been known which completely satisfies the requirements of boundary lubrication of aluminum compositions containing at least 50%, by weight, aluminum.

Unexpectedly, we have found that a mixture of a long chain olefin of at least 10 carbon atoms and an organic polar-containing compound described previously can be used as lubricants between two solid surfaces which move relative to each other, even under high pressure conditions; or in many instances these mixtures of compositions can be used as additives to other well known lubricants to impart improved boundary lubrication characteristics to such lubricants, where at least one surface being lubricated is an aluminum surface. When this mixture of

ingredients is employed in lubricating aluminum surfaces, it is found that the coefficient of friction is greatly reduced and the tendency to gall or seize, particularly under boundary lubrication conditions, is materially reduced and in many instances is completely eliminated. Furthermore, it is found that in addition to the improved lubricating characteristics of our lubricating compositions, the act of one surface moving across another surface in the presence of these lubricants imparts a high polish to the aluminum surface, thereby still further increasing the ease with which our lubricating compositions can contribute to the lubricating act.

In addition to our lubricating compositions being especially adaptable for lubricating relatively moving surfaces at least one surface of which is an aluminum surface, it is also possible to use these lubricating compositions for obtaining improved lubrication of other solid surfaces moving relative to each other, especially when one of these surfaces is a metal used for fabricating structural shapes, for example, iron, molybdenum, silver, copper, beryllium, tungsten, magnesium, titanium, zirconium, chromium, nickel, cobalt, aluminum, tin, etc., and various metal compositions, for example, alloys of the aforesaid metals, of which typical examples are steels, brasses, the various alloys of magnesium, cobalt, zinc, zirconium, beryllium, iron (e.g., stainless steel), etc. The other surface may be the same or different metal, or it may be another solid material for example, wood, molded synthetic resins, laminates, etc., or a special compounded composition, such as, porous metal, graphite, graphite-impregnated metal, soft bearing alloys, e.g., babbitts, etc., or very hard compositions, for example, metal carbides, nitrides, etc.

The fact that our mixture of ingredients may be used as lubricants for these various classes of materials and are particularly useful for lubricating two solid surfaces moving relative to each other where at least one of the surfaces is aluminum, was entirely unexpected and in no way could have been predicted, because the prior art has been of the impression that the usual lubricants and the usual lubricating materials and techniques were not effective lubricants under many conditions for relatively moving parts in which one of the surfaces was aluminum. This was due to the fact that aluminum or alloys of aluminum were relatively soft, and when employing the usual lubricants for aluminum, even extreme pressure lubricants containing additives to increase the load bearing characteristics of lubricant, this resulted in undesirable wear, galling and ultimate seizure of the aluminum comprising the relatively moving parts. This is particularly borne out by a recent article by R. D. Guminski and J. Willis, entitled "Development of Cold-Rolling Lubricants for Aluminum Alloys," in Journal of the Institute of Metals, 88, pages 481—492 (1960) where the authors point out the undesirability of having unsaturated additives as lubricants in the cold-rolling of aluminum alloys.

The long chain olefins which we employ in our invention have the general formula

60 (I)



65 where R and R' are monovalent radicals selected from the class consisting of hydrogen and fluorine, and additionally R' is selected from the class consisting of the methyl, fluoromethyl, difluoromethyl, and trifluoromethyl radicals, and R'' is a monovalent straight chain saturated aliphatic radical selected from the class consisting of linear alkyl radicals having at least 8 carbon atoms and linear fluoroalkyl radicals having at least 8 carbon atoms.

Preferably, R" does not exceed 30 carbon atoms, although longer chain radicals may be used. It will of course be understood that mixtures of these olefins may be employed in the practice of our invention.

The ester component in this particular class of lubricants, which must be free of olefinic unsaturation, comprises a compound having the formula



Z is a monovalent, linear, straight chain saturated aliphatic radical selected from the class consisting of linear alkyl and linear fluoroalkyl radicals of from 11 to as long as 40 carbon atoms or more, X is a divalent radical selected from the group consisting of oxy ( $-O-$ ),



where Z is as previously defined. Q is a monovalent lower alkyl straight chain radical of from 1 to 3 carbon atoms selected from the class consisting of alkyl radicals and fluoroalkyl radicals, e.g., methyl, ethyl, propyl, fluoromethyl, difluoromethyl, trifluoromethyl, 1,2-difluoroethyl, perfluoropropyl, etc.

Included among the normal compounds (as contrasted to branched chain compounds) represented by Formula I are, for instance, decene-1, dodecene-1, tetradecene-1, dodecene-2, tetradecene-2, pentadecene-1, hexadecene-1 (cetene), octadecene-1, octadecene-2, 1-fluorotetradecene-1, 1,2-difluorotetradecene-1, 1-fluorohexadecene-1, 40 trifluorohexadecene-1, 1,1,2,2 - tetrafluorohexadecene-2, etc., as well as mixtures of such olefins.

Among the radicals which Z may be are, for example, undecyl, dodecyl, tetradecyl, hexadecyl, pentadecyl, eicosyl, docosyl, tricosyl, triacontyl, tetracontyl, 1,1,1,2,2-pentafluorotetradecyl, tetrafluorododecyl hexafluorotetradecyl, etc.

Examples of compounds coming within the scope of Formula II are, for instance, methyl laurate, propyl laurate, methyl myristate, methyl palmitate, methyl stearate, ethyl carnaubate, n-propyl myristate, ethyl palmitate, methyl behenate, undecyl acetate, dodecyl acetate, dodecyl propionate, monofluoromethyl stearate, 1,1-difluoroethyl palmitate, trifluoromethyl fluoromyristate, methyl fluoropalmitate, difluoromethyl palmitate, methyl difluorostearate, dodecyl fluoroacetate, fluoromethyl trifluoromyristate, methyl undecyl ether, methyl dodecyl ether, ethyl tetradecyl ether, ethyl eicosyl ether, ethyl hexadecyl sulfide, ethyl undecyl sulfide, propyl dodecyl sulfide, methyl dodecyl ketone, ethyl dodecyl carbonate, methyl tetradecyl sulfoxide, ethyl hexadecyl sulfone, ethyl tetradecyl ether, ethyl eicosyl sulfide, methyl monofluoromonadecyl carbonate, fluoromethyl dodecyl ether, methyl tetrafluorotricosyl sulfone, methyl hexafluorotriacontyl sulfoxide, propyl trifluoroundecyl ketone, ethyl trifluorostearate, 2-fluoroethyl octadecyl sulfide, 1,2-difluoropropyl eicosyl ketone, fluoroethyl tetrafluorotricosyl sulfone, methyl trifluorotricosyl ether, etc.

The proportions of the two ingredients can be varied widely and generally are preferred in such proportions that the combination of the two imparts the desired lubricating characteristics and represents a fluid mixture which has a solidification temperature well below room temperature, for example, below 15° C., thus making the lubricant useful over a broad spectrum of temperatures.

In general, amounts of the olefin as low as 5% in the mixture give significant results. We have found that the olefin component advantageously is present in an amount equal to about 5-95%, by weight, of the total weight of the olefin and the other component represented by Formula II. Obviously, mixtures of the olefins may be used in combination with mixtures of the compounds represented by Formula II.

Because of the ease of preparation, ready availability of raw materials for synthesis and their suitability and outstanding properties as lubricants and as additives to other well known lubricants, we prefer to use as the olefinic component one which is a straight chain unsaturated aliphatic hydrocarbon having olefinic unsaturation in the 1- or 2- positions of a chain length of from 12 to 20 carbon atoms, while the other component of our lubricant conforming to Formula II is advantageously chosen from saturated aliphatic esters of saturated aliphatic monocarboxylic acids in which the saturated aliphatic radical Z is from about 12 to 20 carbon atoms in length.

The above mixture of ingredients can be used alone or can be mixed with other well known lubricants, for example, mineral oils of lubricating viscosity, greases made from such lubricating oils, silicone lubricating oils, diester lubricating oils, polyester lubricating oils, silicate ester lubricating oils, etc. Aqueous emulsions of our lubricating composition, either alone or in combination, with other well known cutting oils can be used to advantage in cutting and grinding applications. Our lubricants are particularly useful in lubricating solid surfaces which move relative to each other where one of the surfaces is aluminum. When one solid surface moves relative to another surface with a lubricant between the two surfaces, there may be a complete film of lubricant separating the two surfaces or there may be varying degrees of contact between the surfaces. The former condition exists under ideal hydrodynamic lubrication, while the latter condition is characteristic of boundary lubrication. Complete hydrodynamic lubrication may be obtained under certain ideal conditions found in bearings but is influenced by such factors as design of the two solid surfaces, load on the surfaces, and the relative speed of one part to the other. However, even under these conditions, boundary lubricating problems are encountered during stopping and starting operations, and from a practical standpoint, perfect hydrodynamic lubrication is approached rather than attained. Therefore, the ability of our lubricants to improve the boundary lubrication of solid surfaces moving relative to each other where one of the surfaces is aluminum, is a feature which has been greatly desired in the past.

In addition to our lubricants improving the lubricating characteristics of two solid surfaces where both surfaces are aluminum, it should also be understood that our lubricants are also useful in those cases where one of the surfaces is aluminum and the other surface is another solid material, as, for instance, various metals, for example, iron, molybdenum, copper, tungsten, magnesium, zirconium, chromium, nickel, etc., alloys of said metals, such as steels, brasses, the alloys of magnesium, cobalt, zirconium, beryllium, aluminum, iron, zinc, etc. In addition, the other surface may be still other solid materials, for example, wood, molded synthetic resins, laminates, etc., or special compounded compositions such as porous metal, graphite, graphite impregnated metal, soft bearing alloys, e.g., babbitts, etc., or very hard compositions, for example, metal carbides, nitrides, etc. The lubrication of the above metals alone other than aluminum, by means of our compositions is not precluded. Thus, the lubrication of surfaces where one of the surfaces is titanium, beryllium, tungsten, etc., useful for fabricating structural shapes is included in the scope of the invention.

Nominally, in the design of equipment where one solid surface moves relative to another, both solid surfaces

are the same material if the wear is to be equal on both parts or one is made of a material softer than the other when the wear is to be essentially all on the softer part. This is usually done when one part is easier to replace than the other or the one part is being cut or shaped by the other.

A concentration of even small amounts, and, for example, at least 15%, by weight, of our compositions in another lubricant, will show significant improvement in the boundary lubricating properties of the latter. Generally, we have found that for a solid surface of aluminum where the other surface moving relative to the first is also aluminum, the coefficient of friction is generally greatly improved where at least 50%, by weight, of the total lubricant constitutes the mixture of the olefinic material and the compound represented by Formula II above. On a weight basis we may use from 10 to 90 parts of our lubricant mixture per 100 parts of the other usual lubricant. For the first time, this discovery permits the use of a wide variety of aluminum compositions in the fabrication of bearings and like surfaces, since, as far as we are aware, prior to our invention, no way was satisfactorily known to prevent galling and seizing of bearings made of aluminum. Although specific alloys of aluminum were made for bearings, the use of such compositions required concessions to be made as to the bearing clearances, life, etc., in order to provide adequate performance.

Likewise, our lubricating compositions permit aluminum materials to be shaped, for example, by drawing, spinning, extrusion and the like, with a very smooth finish. When our materials are used as the lubricant without dilution, the aluminum composition can be formed with a smooth, mirror-like finish which is difficult to obtain by the use of previously known lubricants. Typical examples of the various aluminum compositions (including aluminum alloys) that can be lubricated by our lubricants are those disclosed on pages 851-853 and 865-958 of Metals Handbook, vol. 1, Properties and Selection of Metals, American Society for Metals, Novelty, Ohio, Eighth Edition (1961), for example, the high purity aluminum alloys which are greater than 99% aluminum, e.g., EC alloy, 1060 alloy, 1100 alloy, etc., alloys of aluminum with other metals, for example, copper, silicon, tin, zinc, etc., as are more fully described on pages 955-958 of the above reference.

Typical of the mineral or hydrocarbon oils of lubricating viscosity are the hydrocarbon lubricants obtained from petroleum. These products normally have viscosities in the range of 25 to 10,000 Saybolt Universal Seconds (S.U.S.), and may be a single mixture of hydrocarbons.

Typical of the silicone lubricating oils are those disclosed in, for example, U.S. Patents 2,410,346—Hyde; 2,456,496—Ford et al.; 2,469,888—Patnode; 2,469,890—Patnode; 2,970,162—Brown; etc.

Typical of the diester, polyester, and silicate ester lubricants are those disclosed in U.S. Patents 2,450,221—Ashburn et al.; 2,450,222—Ashburn et al.; U.S. Patent 2,977,301—Bergen et al.; and on pages 16-24 of Technical Publication No. 77, published by American Society for Testing Materials, Philadelphia, entitled, "Symposium on Synthetic Lubricants." Other lubricating materials, as well as suitable mixtures of these lubricating materials, may be used in the practice of our invention without departing from the scope of the invention.

The compositions of our invention covered by the above general formula vary from liquid to solid materials. The solids when dissolved in lubricating oils or fluids are capable of producing fluids and greases having improved lubricating properties depending on the composition and concentration.

To aid in obtaining the grease-like consistency desired for lubricating greases, non-abrasive fillers such as silica gel, carbon black, diatomaceous earth, molybdenum sulfide, tin sulfide, graphite, etc., may be added or soaps may be incorporated to produce a gel structure. Particularly

useful soaps are the metallic soaps such as the alkali or alkaline earth soaps of the fatty acids, but other soaps may also be used, for example, zinc, tin, lead, copper, etc., soaps of the fatty acids. A particularly desirable grease composition may be made from lithium stearate or lithium hydroxy stearate. These grease compositions may be made by any of the well known methods, for example, as disclosed in U.S. Patents 2,450,221—Ashburn et al.; 2,450,222—Ashburn et al.; and 2,260,625—Kistler.

It will of course be apparent to those skilled in the art that in addition, pour depressants, stabilizers, inhibitors, particularly oxidation inhibitors, and the like, may be added to our lubricating compositions to impart to the latter the additional properties which these particular additives are designed for.

In order that those skilled in the art may better understand how the present invention may be practiced, the following examples are given by way of illustration and not by way of limitation. In all of the examples, the percentages are by weight.

The apparatus used to test our lubricants shown in the following examples under boundary lubricating conditions is described in the attached drawing, in which the single figure shows partly in section the portion of a standard four-ball wear tester which has been modified to evaluate lubricating compositions using metals in various shapes other than the balls.

This apparatus comprised a modified four-ball wear test machine described in an article by R. G. Larson, entitled, "Study of Lubrication Using Four-Ball Type Machine," Lubrication Engineering, 1, page 35, August, 1945. This machine was modified by replacing the four balls and their holder with a cup and washer, as shown in the figure. Rider 1, made of aluminum (or another metal), is cup-shaped and is rotated at preselected speeds against stationary test washer 2 made also of aluminum (or another metal) by means of a motor driven shaft 3 to which rider 1 is attached by machine bolts 4 and 4'. Washer 2 is rigidly fastened to the base 5 of chamber 6 by means of machine bolt 7 through the medium of a rubber member designed to insure proper alignment between washer 2 and rider 1. A reservoir of lubricant 8 under test is maintained around the test pieces. Chamber 6 rides on a series of ball bearings, one of which is shown as 9, which ride upon member 10, which forms the uppermost portion of plunger 11, which is connected to a hydraulic system (not shown) to permit various loadings to be established between the two test samples 1 and 2. When rider 1 is rotated against test washer 2 by means of clockwise rotation of shaft 3, chamber 6 will rotate upon member 10 due to the frictional force existing between members 1 and 2. The force required to prevent such rotation is measured by a strain gauge attached to arm 12. This modification permits the coefficient of friction to be calculated and examination of riders 1 and 2 permits evaluation of the amount and type of wear produced.

Using this apparatus, the following measurements were made in the following tests when the rider having a flat annular surface area of 0.393 square inch was rotated at 0.88 r.p.m. to give a surface speed of 0.0461 inch per second against the test washer under of a load of 10 kg. These conditions represent operation in the boundary friction region and represent the most difficult condition of bearing operation from a lubricant standpoint. All percentages are by weight and the tests were run at room temperature (about 22° C.) for one hour unless otherwise specified. In some of the examples below the rider and washer were of materials other than aluminum specifically stainless steel and titanium in order to show the versatility of our lubricants.

#### EXAMPLE 1

In this example, a lubricant mixture consisting of 70% cetene and 30% methyl stearate was introduced in the above-described apparatus in which the rider and washer

were both 403 stainless steel (11.5-13% chromium). The test for the efficiency of the lubricant was conducted for 1.5 hours at the end of which time it was found that the coefficient of friction remained steady at around 0.16. Examination of the wear surface of the washer showed no discernible wear with the exception that it was highly polished. For comparison, when cetene alone was tested under the same conditions using the same stainless steel washer and rider the coefficient of friction was quite erratic and showed a wide scatter between 0.27 and 0.4. In addition, the surface of the washer showed deep grooving indicating excessive wear.

## EXAMPLE 2

In the following example, mixtures of cetene (made and sold by Matheson, Coleman and Bell of East Rutherford, New Jersey) (also known as hexadecene-1) and methyl stearate and a mixture of n-decene-1 and methyl stearate in the proportions stipulated were introduced as the lubricant mixture in the above-identified apparatus in which the rider and washer were both aluminum. Additionally, cetene alone (methyl stearate a solid at room temperature) and cetane alone, were also tested for comparison purposes to show the unexpected advantages of using the combination of an olefinic hydrocarbon and a composition conforming to Formula II. In addition to evaluating the effect of using the foregoing compositions as lubricants in the above described test apparatus, mixtures of cetene with either n-butyl stearate or isopropyl stearate were also evaluated. Finally, a vegetable oil (corn oil) was tested to show the effect of having polyunsaturation in one ester molecule. This vegetable oil consisted essentially of glycerides of fatty acids containing, on a weight basis, acid residues of the following acids; 34 to 62% linoleic acid, 19 to 49% oleic acid, 0.2 to 1.6% hexadecenoic acid, 8 to 12% palmitic acid, and less than 5% of small amounts of myristic and stearic acids. The 150 SUS hydrocarbon oil was a mineral lubricating oil of 150 Saybolt units viscosity widely employed as a lubricant for bearing surfaces. Table 1 shows the compositions of the test lubricants, the proportions of the lubricants and remarks as to the type of wear encountered in each instance.

Table 1

| Lubricant                                     | Average Coefficient of Friction | Remarks as to Wear Surface                                        |
|-----------------------------------------------|---------------------------------|-------------------------------------------------------------------|
| 100% cetene                                   | 0.11                            | Very high wear as though the surface were machined. Galled badly. |
| Vegetable Oil <sup>1</sup>                    | 0.27-0.38                       | Very little wear after 1 hour.                                    |
| 20% methyl stearate, 80% cetene               | 0.1                             | Polished surface; No visible wear.                                |
| 30% methyl stearate, 70% cetene               | 0.1                             | Do.                                                               |
| 40% methyl stearate, 60% cetene               | 0.1                             | Do.                                                               |
| 50% methyl stearate, 50% cetene               | 0.09                            | Do.                                                               |
| 30% methyl stearate, 70% n-decene-1           | 0.11                            | Do.                                                               |
| 30% isopropyl stearate, 70% cetene            | 0.1-0.24                        | Grooved and galled in 40 minutes.                                 |
| 20% n-butyl stearate, 80% cetene <sup>1</sup> | 0.14-0.4                        | Grooved and galled badly.                                         |
| 50% n-butyl stearate, 50% cetene <sup>1</sup> | 0.12-0.34                       | Badly galled.                                                     |
| 100% 150 SUS hydrocarbon oil <sup>1</sup>     | 0.2-0.7                         | Galled.                                                           |
| 20% methyl stearate, 80% 150 SUS oil          | 0.2-0.25                        | Do.                                                               |
| 100% cetane <sup>1</sup>                      | 0.4->0.68                       | Galled badly, seized.                                             |
| 30% methyl stearate, 70% cetane               | 0.14                            | Galled.                                                           |

<sup>1</sup> At all times during the test, the coefficient of friction was erratic and varied within the limits set forth.

## EXAMPLE 3

In this example employing the lubricating test equipment described above in which both the rider and the washer were made of titanium, a mixture of 70% cetene and 30% methyl stearate were introduced as the lubricant mixture in the apparatus. For comparison and as a control a hydrocarbon oil specifically SAE-10 spindle oil was used as a lubricant under the same conditions. After

conducting the wear test, it was found that the average coefficient of friction using the spindle oil was quite erratic and ranged from about 0.56-0.68; the test disc or washer was badly galled and caused grooving during the 1-hour run. In contrast to this employing the mixture of cetene and methyl stearate, the average coefficient of friction was of the order of about 0.5-0.6 and the washer showed only a very slight wear track.

## EXAMPLE 4

When a mixture of 50% tetradecene-2 is mixed with 30% ethyl tetradecyl ether and this mixture is employed as a lubricant between two surfaces of aluminum that is both the rider and washer were aluminum in the above test equipment, the coefficient of friction is much lower by a magnitude in kind and the wear is materially reduced than when either the aforesaid ether or tetradecene is used separately as the lubricant. The wear is also much less than when a hydrocarbon oil is employed as the lubricant.

It will be clearly apparent that our compositions can be used not only in bearing applications where a shaft, for instance, is revolving in intimate contact with a stationary member, but they can also be employed in other applications as, for instance, in the cutting of aluminum, the extrusion, drawing and stamping of aluminum members, etc. Aluminum cans can be readily drawn to be used for capacitor casings. Furthermore, billets of aluminum can be passed through dies and the diameter of the billets greatly reduced in size to give aluminum wire which has a shiny appearance and, because of the smooth surfaces of the aluminum, reflects the advantageous lubricating characteristics of our lubricating compositions. This ability to impart smooth shiny surfaces recommends these compositions as polishing materials for sole plates of sadirons. Fractional horsepower motors (such as those described in our copending application Serial No. 101,917, filed April 10, 1961, and in the continuation-in-part filed concurrently herewith based on that application, which by reference are made part of the disclosures of the instant application), using aluminum shafts and bearings can be advantageously lubricated with our lubricating compositions either alone or dissolved to the desired concentration in a hydrocarbon lubricating oil.

It will also be apparent to those skilled in the art that, instead of the particular olefins and the methyl stearate used in the foregoing tests, other olefins and compounds conforming to Formula I and Formula II may be used without departing from the scope of the invention. The proportions of ingredients can of course be varied widely, and it will also be obvious that other lubricating compositions, many examples of which have been given above, can be combined with our mixture of ingredients comprising the olefinic compound and the compounds of Formula II to give compositions of matter having utility in the lubricating art, particularly under boundary lubricating conditions.

What we claim as new and desire to secure by Letters Patent of the United States is:

1. A composition of matter comprising on a weight basis (a) from 5 to 95% of an olefin having the formula



and (b) from 95 to 5% of a compound having the formula



where R is a monovalent radical selected from the class consisting of hydrogen and fluorine, R' is a monovalent radical selected from the class consisting of hydrogen, fluorine, methyl, monofluoromethyl, difluoromethyl, and trifluoromethyl, R'' is a monovalent linear, straight-chain alkyl radical selected from the class consisting of linear

alkyl and linear fluoroalkyl radicals having from 8 to 30 carbon atoms, X is a divalent radical selected from the group consisting of  $-\text{O}-$ ,  $-\text{S}-$ ,



and Z is a monovalent linear straight-chain saturated aliphatic radical selected from the group consisting of linear alkyl radicals having from 11 to 40 carbon atoms and linear fluoroalkyl radicals having from 11 to 40 carbon atoms, and Q is a lower, straight-chain alkyl radical of from 1 to 3 carbon atoms.

2. A lubricating composition of matter comprising by weight, from 5 to 95% methyl stearate and from 95 to 5% cetene.

3. A lubricating composition of matter comprising, by weight, from 5 to 95% methyl stearate and from 95 to 5% decene-1.

4. A lubricant composition of matter comprising, by weight, from 5 to 95% ethyl tetradecyl ether and from 95 to 5% tetradecene-2.

5. A lubricating composition comprising a mixture of ingredients containing, on a weight basis, (1) 100 parts of a lubricating fluid selected from the class consisting of silicone, diester, hydrocarbon, polyester, and silicate ester lubricating fluids, and (2) from 10 to 90 parts of a mixture of ingredients comprising on a weight basis (a) from 5 to 95% of an olefin having the formula



and (b) from 95 to 5% of a compound having the formula



where R is a monovalent radical selected from the class consisting of hydrogen and fluorine, R' is a monovalent radical selected from the class consisting of hydrogen fluorine, methyl, monofluoromethyl, difluoromethyl, and trifluoromethyl, R'' is a monovalent linear straight-chain alkyl radical selected from the class consisting of linear alkyl and linear fluoroalkyl radicals having from 8 to 30 carbon atoms, X is a divalent radical selected from the group consisting of  $-\text{O}-$ ,  $-\text{S}-$



and



and Z is a monovalent linear straight-chain saturated aliphatic radical selected from the group consisting of linear alkyl radicals having from 11 to 40 carbon atoms and linear fluoroalkyl radicals having from 11 to 40 carbon atoms, and Q is a lower, straight-chain alkyl radical of from 1 to 3 carbon atoms.

6. A lubricating composition comprising a mixture of ingredients containing, on a weight basis (1) 100 parts of a lubricating fluid selected from the class consisting of silicone, diester, hydrocarbon, polyester, and silicate ester lubricating fluids, and (2) from 10 to 90 parts of a mixture of ingredients comprising on a weight basis (a) from 5 to 95% methyl stearate, and (b) from 95 to 5% cetene.

7. The method of lubricating two solid surfaces between which there is relative motion, at least one of said surfaces being a metal, which comprises maintaining between the two surfaces a composition of matter com-

prising on a weight basis (a) from 5 to 95% of an olefin having the formula



and (b) from 95 to 5% of a compound having the formula



where R is a monovalent radical selected from the class consisting of hydrogen and fluorine, R' is a monovalent radical selected from the class consisting of hydrogen fluorine, methyl, monofluoromethyl, difluoromethyl, and trifluoromethyl, R'' is a monovalent linear, straight-chain alkyl radical selected from the class consisting of linear alkyl and linear fluoroalkyl radicals having from 8 to 30 carbon atoms, X is a divalent radical selected from the group consisting of  $-\text{O}-$ ,  $-\text{S}-$



and Z is a monovalent linear straight-chain saturated aliphatic radical selected from the group consisting of linear alkyl radicals having from 11 to 40 carbon atoms and linear fluoroalkyl radicals having from 11 to 40 carbon atoms, and Q is a lower, straight-chain alkyl radical of from 1 to 3 carbon atoms, and thereafter effecting motion between the two solid surfaces with the mixture of ingredients therebetween.

8. The method of lubricating two solid surfaces between which there is relative motion, at least one of said surfaces being a metal selected from the class consisting of aluminum and alloys of aluminum, which comprises maintaining between the two surfaces a mixture of ingredients comprising on a weight basis (a) 5 to 95% methyl stearate and (b) from 95 to 5% cetene, and thereafter effecting motion between the two solid surfaces with the mixture of ingredients therebetween.

9. The method of lubricating two solid surfaces between which there is relative motion, at least one of said surfaces being a metal selected from the class consisting of aluminum and alloys of aluminum, which comprises maintaining between the two surfaces a mixture of ingredients comprising on a weight basis (a) 5 to 95% methyl stearate and (b) from 95 to 5% decene-1, and thereafter effecting motion between the two solid surfaces with the mixture of ingredients therebetween.

10. The method of lubricating two solid surfaces between which there is relative motion, at least one of said surfaces being aluminum, which comprises maintaining between the two surfaces a mixture of ingredients comprising on a weight basis (a) 5 to 95% ethyl tetradecyl ether and (b) from 95 to 5% tetradecene-2, and thereafter effecting motion between the two surfaces with the mixture of ingredients therebetween.

11. The process for shaping a metal composition which comprises maintaining a film of lubricant between the metal composition and a shaping member, said lubricant comprising on a weight basis (a) from 5 to 95% of an olefin having the formula



and (b) from 95 to 5% of a compound having the formula



where R is a monovalent radical selected from the class consisting of hydrogen and fluorine, R' is a monovalent radical selected from the class consisting of hydrogen fluorine, methyl, monofluoromethyl, difluoromethyl, and trifluoromethyl, R'' is a monovalent linear, straight-chain alkyl radical selected from the class consisting of linear

## 11

alkyl and linear fluoroalkyl radicals having from 8 to 30 carbon atoms, X is a divalent radical selected from the group consisting of  $-\text{O}-$ ,  $-\text{S}-$ ,



and Z is a monovalent linear straight-chain saturated aliphatic radical selected from the group consisting of linear alkyl radicals having from 11 to 40 carbon atoms and linear fluoroalkyl radicals having from 11 to 40 carbon atoms, and Q is a lower, straight-chain alkyl radical of from 1 to 3 carbon atoms, and thereafter subjecting the metal composition to sufficient force to create relative motion between said metal composition and said shaping member and to cause displacement of a portion of said metal composition with respect to the remainder thereof.

## 12

12. The process as in claim 11 in which the metal composition undergoing shaping is an aluminum composition selected from the class consisting of aluminum and alloys of aluminum of which 50%, by weight, is aluminum, and the lubricant is a mixture comprising, by weight, from 5 to 95% cetene and from 95 to 5% methyl stearate.

## References Cited by the Examiner

## UNITED STATES PATENTS

|    |           |       |                |             |
|----|-----------|-------|----------------|-------------|
| 10 | 2,210,140 | 8/40  | Colbeth        | 252—56      |
|    | 2,257,969 | 10/41 | Loane et al.   | 252—48.2    |
|    | 2,500,165 | 3/50  | Doherty et al. | 252—59 XR   |
|    | 2,659,252 | 11/53 | Kipp           | 252—11 XR   |
| 15 | 2,729,992 | 1/56  | Wankat         | 252—51.5 XR |

DANIEL E. WYMAN, Primary Examiner.